

## UNITED STATES PATENT OFFICE

2,521,106

METHOD AND BATH FOR  
ELECTROPOOLISHING

Harold J. Wiesner, Elkhart, Ind., assignor to C. G. Conn, Ltd., Elkhart, Ind., a corporation of Indiana

No Drawing. Application January 19, 1946,  
Serial No. 642,435

16 Claims. (Cl. 204—140.5)

1

This invention relates to a method of and bath for electropolishing, and more particularly to the electropolishing of copper and copper alloys.

One of the objects of the invention is to provide a method of and bath for electropolishing in which all of the exposed surfaces of an article to be polished will be given a uniform bright finish free from discoloration.

Another object is to provide a method of and bath for electropolishing copper alloys containing lead which will produce a high luster free from smut.

Still another object is to provide a method of and bath for electropolishing in which the bath is mildly alkaline.

A further object is to provide an electropolishing bath which is non-corrosive so that relatively inexpensive equipment can be used, which is harmless to operators either from contact or from fumes and which requires no venting equipment.

According to the present invention, articles to be polished, which may be any shape or configuration of metal articles formed of copper or copper containing alloys, are connected as an anode in the polishing bath and have a current passed through them to a cathode in the bath which is preferably copper or plated with copper. With the bath of the present invention current densities substantially in excess of 100 amperes per square foot can be used to produce a uniform high luster over the entire surface of the articles, including recessed portions. The time required to produce a brilliant surface is dependent upon the finish of the article prior to the electropolishing operation. It is apparent that for this reason no specific time for accomplishing the electro-polishing to a high luster can be given, but in general the time will vary from 5 to 30 minutes, and on an average will be about 15 to 20 minutes.

The bath of this invention consists essentially of pyrophosphates of the alkali metals and either borates or carbonates mixed therewith in an aqueous solution. The most satisfactory pyrophosphates are sodium pyrophosphate, which is preferably used in the anhydrous or deca-hydrate, and potassium pyrophosphate, which is preferably the trihydrate. These salts function in the solution to form soluble compounds with the copper, zinc, and lead and other metals commonly found in the brass alloys during electro-polishing. In the operation of the bath the copper plates out as a sludge at the cathode so that the net loss of pyrophosphate is that which combines with the zinc, lead and other metals. The bath can therefore be used for relatively long periods of time with the addition of only very small amounts, if any, of pyrophosphates to maintain its strength. I have found that a satisfactory concentration is on the order of 16 ounces

of a pyrophosphate salt per gallon, although this concentration is not critical, and the bath will function satisfactorily with a concentration of pyrophosphate as low as 8 ounces per gallon, or up to its saturation point.

The effect of the borates and carbonates in the bath is to broaden the current density range and to obtain uniformity of polishing. If these materials are omitted there will be substantially less brightening in the recesses of the work and other low current density areas, and etching may occur. Also, discolorations may occur in various areas of the work pieces. Among the specific compounds which I have found to be most satisfactory are boric acid, sodium tetraborate, potassium tetraborate, ammonium carbonate, sodium bicarbonate, and potassium bicarbonate, which are preferably used in concentrations of from 2 to 12 ounces per gallon. If ammonium carbonate is used, it is necessary to keep the temperature of the bath below about 135° F., as above this temperature it decomposes rapidly. Ammonium carbonate and sodium and potassium bicarbonate also react with acid, which may be added to the bath to lower its pH to give off some carbon dioxide. Boric acid and sodium or potassium tetraborate are preferred since they are thermally stable, do not decompose when acid is added, and function to buffer the solution.

In addition to these basic constituents of the bath there may be added either an acid or base in quantities sufficient to bring the pH of the bath in the range from 7.5 to 9.5. For this purpose sodium, potassium or ammonium hydroxide may be conveniently used to raise the pH, while sulfuric or meta phosphoric, and in some cases ortho phosphoric, acid may be used to lower the pH. If the pH of the bath is below about 7.5, the satisfactory current density range is substantially narrowed, while if the pH is too high, a highly lustrous surface cannot be obtained. More specifically, if the pH drops below the aforementioned lower limit and electropolishing is attempted on a complicated piece of work, it has been found that brown to reddish-brown discolorations will be apparent on the high current density areas. As the pH of the solution is raised (with sodium hydroxide, for example) the current density range is broadened, and at a pH of 9.0 (for example) extremely high current densities may be used without burning.

In baths containing ammonium carbonate, sodium hydroxide may be used satisfactorily to raise the pH, but in those baths containing boric acid or sodium tetraborate, ammonium hydroxide or an ammonium compound was found to give better results. To lower the pH sulphuric, meta-phosphoric or ortho-phosphoric acids may be used satisfactorily but certain other acids

## 3

such hydrochloric have been found not to produce good results.

The current density range may be further extended and greatly increased brightness produced by the addition of orthophosphate salts to the bath. Examples of satisfactory salts are sodium, ammonium or potassium salts such as mono, di or tri sodium or potassium phosphate and mono or di ammonium phosphate. The di sodium, di potassium and di ammonium phosphates, when put into solution, have pH values nearer to those in the operating range of the bath and for this reason are preferred. These salts, when added to the bath in concentrations of from 12 to 20 ounces per gallon extend the current range and greatly increase brightness.

It has further been found that the addition of oxalic acid or one of its salts such as sodium oxalate, ammonium oxalate or potassium oxalate in concentrations of about 4 to 6 ounces per gallon enables the temperature of the bath to be increased up to as much as 200° F. with good results. Without the addition of these materials, it has been found that the surface tends to become irregular at temperatures substantially in excess of 150° F.

In general, I have found that agitation of the work or of the solution during electropolishing is desirable. As a result of using agitation, higher current densities are permitted, with less chance of "burning" the protruding sections of a complicated piece of work. The commonly employed methods of agitation used in the electroplating industry, such as oscillation of the work rod, air agitation, or solution agitation by means of pumps or paddles are satisfactory. The use of work rod oscillation is perhaps to be preferred.

As examples of several baths which I have found to be satisfactory, the following may be given:

## Example #1

Sodium pyrophosphate (anhydrous) 16 oz./gal.  
Boric acid 5 oz./gal.  
Ammonium hydroxide (28° Bé.) 2 fl. oz./gal.  
pH 8.5-9.0  
Temperature 140-160° F.  
Current density Above 100 amps./sq. ft.

## Example #2

Potassium pyrophosphate 16 oz./gal.  
Boric acid 4-6 oz./gal.  
pH 8.5-9.0  
Temperature 140-160° F.  
Current density Above 100 amps./sq. ft.

## Example #3

Potassium pyrophosphate 16 oz./gal.  
Di potassium hydrogen phosphate 5-12 oz./gal.  
Boric acid 4-6 oz./gal.  
pH 8.0-8.5  
Temperature 140-160° F.  
Current density Above 100 amps./sq. ft.

## Example #4

Sodium pyrophosphate (anhydrous) 16 oz./gal.  
Disodium hydrogen phosphate 12-20 oz./gal.  
Boric acid 5 oz./gal.  
pH 8.0-8.5  
Temperature 130°-150° F.  
Current density Above 150 amps./sq. ft.

## 4

## Example #5

Sodium pyrophosphate 16 oz./gal.  
Boric acid 5 oz./gal.  
Sodium oxalate or  
oxalic acid 4-6 oz./gal.  
pH 8.0-8.5  
Temperature 180°-200° F.  
Current density Above 150 amps./sq. ft.

While the invention has been particularly described in connection with several specific bath compositions, it will be understood that various combinations and concentrations of the constituents mentioned, as well as various operating conditions might be employed within the scope of the invention. The examples given are to be taken as illustrative only, reference being had to the appended claims for a determination of the scope of the invention.

What is claimed is:

1. The method of electropolishing copper and alloys of copper comprising connecting the part to be polished as the anode in a bath consisting essentially of water as the solvent, an alkali metal salt present in an amount ranging from 8 ounces per gallon of solution to a saturated solution of the salt, and from 2-12 ounces per gallon of solution of a water soluble salt selected from the group consisting of boric acid, water soluble salts of boric acid and water soluble salts of carbonic acid.

2. The method of electropolishing copper and alloys of copper comprising connecting the part to be polished as the anode in a bath consisting essentially of water as the solvent, an alkali metal salt present in an amount ranging from 8 ounces per gallon of solution to a saturated solution of the salt, and from 2-12 ounces per gallon of solution of a water soluble salt selected from the group consisting of boric acid, water soluble salts of boric acid and water soluble salts of carbonic acid, and maintaining the bath between a pH of 7.5 to 9.5.

3. The method of electropolishing copper and alloys of copper comprising connecting the part to be polished as the anode in a bath consisting essentially of water as the solvent, an alkali metal salt present in an amount ranging from 8 ounces per gallon of solution to a saturated solution of the salt, and from 2-12 ounces per gallon of solution of a water soluble salt selected from the group consisting of boric acid, water soluble salts of boric acid and water soluble salts of carbonic acid, and operating the bath at a temperature of between 100-212° F. and at a current density of in excess of 100 amperes per square foot.

4. The method of electropolishing copper and alloys of copper comprising connecting the part to be polished as the anode in a bath consisting essentially of water as the solvent, an alkali metal salt present in an amount ranging from 8 ounces per gallon of solution to a saturated solution of the salt, and from 2-12 ounces per gallon of solution of a water soluble salt selected from the group consisting of boric acid, water soluble salts of boric acid and water soluble salts of carbonic acid, and operating the bath at a pH of 7.5-9.5, at a temperature between 100° F.-212° F., and at a current density in excess of 100 amperes per square foot.

5. A composition for providing an electropolishing bath when dissolved in water, the ingredients being present in the following proportions per 75 each gallon of solution to be made, said com-

position consisting essentially of an alkali metal pyrophosphate present in an amount ranging from 8 ounces to the saturation point per gallon of solution, 2-12 ounces of a water soluble compound selected from the group consisting of boric acid, water soluble salts of boric acid and water soluble salts of carbonic acid, and from 12-20 ounces of a salt of ortho phosphoric acid in which the metal component is selected from the group consisting of ammonia, sodium and potassium.

6. An electropolishing bath consisting essentially of water as the solvent, an alkali metal pyrophosphate present in an amount ranging from 8 ounces per gallon of solution to an amount saturating the bath, from 2-12 ounces per gallon of solution of a water soluble compound selected from the group consisting of boric acid, water soluble salts of boric acid, and water soluble salts of carbonic acid and from 12-20 ounces of a salt of ortho phosphoric acid in which the metallic component is selected from the group consisting of sodium, potassium and ammonium.

7. A composition for providing an electropolishing bath when dissolved in water, the ingredients of which are present in the following proportions for each gallon of solution, said composition consisting essentially of an alkali metal pyrophosphate present in an amount ranging from 8 ounces to an amount to maintain saturated solution, 2-12 ounces of a water soluble compound selected from the group consisting of boric acid and water soluble salts of carbonic acid, a neutralizing agent in an amount to adjust the pH of the solution to between 7.5 and 9.5, and from 12-20 ounces of a salt of ortho phosphoric acid in which the metallic component is selected from the group consisting of ammonium, sodium and potassium.

8. An electropolishing bath consisting essentially of water as the solvent, an alkali metal pyrophosphate present in an amount ranging from 8 ounces per gallon of solution to an amount saturating the bath, from 2-12 ounces per gallon of solution of a water soluble compound selected from the group consisting of boric acid, water soluble salts of boric acid and water soluble salts of carbonic acid, a neutralizing agent present in an amount to adjust the pH of the bath between 7.5-9.5, and from 12-20 ounces of a salt of ortho phosphoric acid in which the metallic component is selected from the group consisting of ammonium, sodium, and potassium.

9. An electropolishing bath consisting essentially of water as the diluent, an alkali metal pyrophosphate present in an amount ranging from 8 ounces per gallon of solution to a saturated solution of the salt, and from 2-12 ounces per gallon of solution of a water soluble compound selected from the group consisting of boric acid, salts of boric acid, salts of carbonic acid, and from 4-6 ounces per gallon of a water soluble material selected from the group consisting of oxalic acid and water soluble salts of oxalic acid.

10. A composition for providing an electropolishing bath when dissolved in water, the ingredients being present in the following proportions per each gallon of solution to be made, said composition consisting essentially of an alkali metal pyrophosphate present in an amount ranging from 8 ounces to an amount to maintain a saturated solution of the salt in water, and from 2-12 ounces of a water soluble compound selected from the group consisting of boric acid, water

soluble salts of boric acid, water soluble salts of carbonic acid, and from 4-6 ounces per gallon of a water soluble material selected from the group consisting of oxalic acid and water soluble salts of oxalic acid.

11. A composition for providing an electro-polishing bath when dissolved in water, the ingredients being present in the following proportions per each gallon of solution to be made, said composition consisting essentially of an alkali metal pyrophosphate present in an amount ranging from 8 ounces to the saturation point per gallon of solution, 2-12 ounces of a water soluble compound selected from the group consisting of boric acid, water soluble salts of boric acid and water soluble salts of carbonic acid, a neutralizing agent in an amount to adjust the pH to between 7.5-9.5, and from 4-6 ounces per gallon of a water soluble material selected from the group consisting of oxalic acid and water soluble salts of oxalic acid.

12. A composition for providing an electro-polishing bath when dissolved in water, the ingredients being present in the following proportions per each gallon of solution to be made, said composition consisting essentially of an alkali metal pyrophosphate present in an amount ranging from 8 ounces to the saturation point per gallon of solution, 2-12 ounces of a water soluble compound selected from the group consisting of boric acid, water soluble salts of boric acid and water soluble salts of carbonic acid, from 12 to 20 ounces of a salt of ortho phosphoric acid in which the metal component is selected from the group consisting of ammonia, sodium, and potassium, and from 4-6 ounces per gallon of a water soluble material selected from the group consisting of oxalic acid and water soluble salts of oxalic acid.

13. An electropolishing bath consisting essentially of water as the solvent, an alkali metal pyrophosphate present in an amount ranging from 8 ounces per gallon of solution to an amount saturating the bath, from 2-12 ounces per gallon of solution of a water soluble compound selected from the group consisting of boric acid, water soluble salts of boric acid, and water soluble salts of carbonic acid, from 12-20 ounces of a salt of ortho phosphoric acid in which the metallic component is selected from the group consisting of sodium, potassium and ammonium, and from 4-6 ounces per gallon of a water soluble material selected from the group consisting of oxalic acid and water soluble salts of oxalic acid.

14. A composition for providing an electropolishing bath when dissolved in water, the ingredients of which are present in the following proportions for each gallon of solution, said composition consisting essentially of an alkali metal pyrophosphate present in an amount ranging from 8 ounces to an amount to maintain saturated solution, 2-12 ounces of a water soluble compound selected from the group consisting of boric acid and water soluble salts of carbonic acid, a neutralizing agent in an amount to adjust the pH of the solution to between 7.5 and 9.5, from 12-20 ounces of a salt of ortho phosphoric acid in which the metallic component is selected from the group consisting of ammonium, sodium and potassium, and from 4-6 ounces per gallon of a water soluble material selected from the group consisting of oxalic acid and water soluble salts of oxalic acid.

15. An electropolishing bath consisting essentially of water as the solvent, an alkali metal

pyrophosphate present in an amount ranging from 8 ounces per gallon of solution to an amount saturating the bath, from 2-12 ounces per gallon of solution of a water soluble compound selected from the group consisting of boric acid, water soluble salts of boric acid and water soluble salts of carbonic acid, a neutralizing agent present in an amount to adjust the pH of the bath between 7.5-9.5, from 12-20 ounces of a salt of ortho phosphoric acid in which the metallic component is selected from the group consisting of ammonium, sodium, and potassium, and from 4-6 ounces per gallon of a water soluble material selected from the group consisting of oxalic acid and water soluble salts of oxalic acid.

16. The method of electropolishing copper and alloys of copper comprising connecting the part to be polished as the anode in a bath consisting essentially of water as the solvent, an alkali metal pyrophosphate present in an amount ranging from 8 ounces per gallon of solution to an amount saturating the bath, from 2-12 ounces per gallon of a water soluble salt selected from the group consisting of boric acid, water soluble salts of boric acid and water soluble salts of carbonic acid, 12-20 ounces per gallon of solution of a salt

5 of ortho phosphoric acid in which the metallic component is selected from the group consisting of ammonium, sodium and potassium, from 4-6 ounces per gallon of solution of a water soluble material selected from the group consisting of oxalic acid and water soluble salts of oxalic acid, maintaining the bath at a pH between 7.5 and 9.5 and at a temperature between 100-212° F. and operating the bath at a current density in excess of 100 amperes per square foot.

10 HAROLD J. WIESNER.

#### REFERENCES CITED

15 The following references are of record in the file of this patent:

#### UNITED STATES PATENTS

|    | Number    | Name      | Date           |
|----|-----------|-----------|----------------|
| 20 | 2,093,927 | Preston   | Sept. 21, 1937 |
|    | 2,326,950 | Kepfer    | Aug. 17, 1943  |
|    | 2,330,170 | Manuel    | Sept. 21, 1943 |
|    | 2,428,141 | Burkhardt | Sept. 30, 1947 |

#### FOREIGN PATENTS

|    | Number  | Country       | Date          |
|----|---------|---------------|---------------|
| 25 | 513,530 | Great Britain | Mar. 31, 1939 |